

Jan. 14, 1936.

E. H. CAMERON

2,027,957

STIFFENING MATERIAL

Filed Aug. 19, 1933

Highly Porous Deposit of Precipitated Colloidal  
Material e. g. Cellulose Ester



More Colloided and More Solvent Resistant Colloidal  
Material e. g. Cellulose Ester

INVENTOR  
EARLE H. CAMERON

BY *Donald G. Ferguson*  
his ATTORNEY

## UNITED STATES PATENT OFFICE

2,027,957

## STIFFENING MATERIAL

Earle H. Cameron, Caldwell, N. J., assignor to  
The Celastic Corporation, Wilmington, Del., a  
corporation of Delaware

Application August 19, 1933, Serial No. 685,909

13 Claims. (Cl. 12—146)

This invention relates to stiffening material and particularly to an improved material of the general type disclosed in United States Patent 1,256,240, Lovell, February 12, 1918. Although not restricted to such use, material of the present type finds advantageous application as stiffening material for boots and shoes, such as fabric, patent leather, cut-out, or perforated boots and shoes, and therefore is described with more particular reference to the boot and shoe industry.

Material of the Lovell type comprises a base fabric such as a woven material, for example cotton cloth, or a structureless material, for example felt or paper, with its interstices carrying a precipitated colloidal material in a highly porous form termed "powdered" by Lovell, such as a cellulosic derivative, casein, albumin and various gum and resins. In use, the fabric is immersed in a solvent for the precipitated material, thereby to resolve the same into a coalescent flaccid condition, and when the material is in this condition the fabric is applied in the lasting operations, shaped, and allowed to harden, by evaporation of solvent, in its shaped condition. While material of the Lovell type is highly satisfactory in use, it sometimes gives rise to the difficulty that the colloidal matter becomes so soft and mushy when the stiffener is dipped into the solvent, that the colloidal matter can be forced through the upper of a shoe of fabric or similar material, during the lasting operations, thereby staining, disfiguring and ruining the upper; and similarly, the coating on a patent leather shoe upper will be affected and softened during the lasting operations so that the coating will be peeled from the leather, thereby damaging the upper; and, again, in lasting shoes having cut-outs or perforations in the upper, the colloidal matter may be forced through the cut-outs or perforations.

I have now devised a stiffening material of the general Lovell type which, in itself, overcomes the difficulties mentioned, and have also devised a method for the manufacture of such material.

In the accompanying drawing, the figure is a highly conventional exaggerated cross sectional view of stiffening material made in accordance with the present invention and embodying the present invention.

One object of my invention is to provide a stiffening material of the mentioned and other desirable characteristics. A further object is to provide a method for the production of such ma-

terial. To these ends, and also to improved generally on materials and methods of the general character indicated, my invention consists in the various matters hereinafter described and claimed.

These objects are accomplished by treating the stiffening material of the Lovell type, and therefore having its entire content of colloidal material in precipitated form, in such a way that the colloidal material is dissolved (although not permanently removed from the fabric) and then re-deposited (or attached) on the fabric in such a way that a part of the deposit is in colloidal form, as distinguished from a precipitated form, but the remainder of the deposit is in a precipitated form. As the colloidal matter, in the fabric after treatment, is not entirely in a precipitated or highly porous condition, it does not absorb the solvent, with which the fabric is ultimately treated for its use in the lasting operation, as quickly or in such a large amount as would the ordinary Lovell material and, therefore, does not become as mushy as would the original material. Yet, on the other hand, it will absorb enough solvent so that it will soften quicker than material prepared merely by subjecting a fabric impregnated with a cellulosic derivative dope to an air drying operation, e. g. that type of material known as the "air dried colloided stiffener". Thus the present material overcomes the disadvantages of the ordinary stiffening material with precipitated colloidal matter while retaining the fundamental advantages of such material.

Specifically, the stiffening material is treated in a solvent bath containing a precipitation-restraining agent that is immiscible or but partially miscible in a following bath in which the material is to be immersed for the purpose of precipitating colloidal material dissolved by the first bath. The said agent may be either a solvent or a non-solvent for the colloidal material. Whether the agent be a solvent or a non-solvent, its primary characteristic is that it is immiscible or at most only partially miscible with the precipitating bath, as otherwise there would be complete precipitation in the following bath.

When the solvent bath is composed of only a single ingredient, this ingredient must not only be a restraining agent but must also be a solvent and be partially miscible in the following bath. When the solvent bath comprises more than one ingredient, the restraining agent need not be a solvent, provided one of the other ingredients present is a solvent; and, furthermore this in-

5 gredient that is a solvent may be entirely miscible in the following bath since the agent furnishes the factor of immiscibility called for. The precipitating liquid in the precipitating following bath tends to immediately and completely displace the solvent-bath liquid to the extent that that liquid is miscible in the following bath; but, to the extent that that liquid is immiscible in the following bath it restrains its own immediate or complete displacement, and thereby to that extent prevents the precipitation of a part of the colloidal matter.

10 After treatment, the fabric is dried, e. g. air dried, whereupon that part of the colloidal matter whose precipitation has been prevented and which has consequently been deposited during the process of air drying by evaporative removal of solvent therefrom, will be in a harder and more colloided form than before treatment.

15 20 In the use of the fabric, blanks of suitable shape may be cut therefrom. These are dipped into a suitable solvent, e. g. diacetone alcohol and ethyl alcohol which will render the blank soft enough to conform to the desired shape. The colloidal matter is re-dissolved, into a coalescent flaccid body which may be placed and conformed into the desired shape and will dry in the desired shape, stiff, flexible and resilient.

25 30 The particular colloidal matter and the stiffener to which the present invention is applicable may be, as above indicated, of many general types. When of cellulosic derivative, it may be of cellulose ester, e. g. cellulose nitrate or cellulose acetate, or cellulose ether, e. g. ethyl cellulose or benzyl cellulose. The solvent for treatment in particular accordance with the present invention will, of course, be selected for compatibility with the particular colloid in question.

35 40 For example, for the production of goods in accordance with the invention, a Lovell material carrying cellulose nitrate in precipitated form may be treated with a bath of (by volume) ethyl alcohol 90% and castor oil 10%, and the precipitating bath be water since the castor oil is immiscible therewith. Material carrying cellulose acetate or cellulose nitrate in precipitated form may be treated with a bath of (by volume) acetone 80% and toluol 20% and the precipitating bath be water since the toluol is nearly immiscible therein. Material carrying cellulose acetate or cellulose nitrate in precipitated form may be treated with a bath of (by volume) acetone 80% and ethyl acetate 20% and the precipitating bath be water since the ethyl acetate is only partially miscible in the said bath. Material carrying cellulose acetate or cellulose nitrate in precipitated form may be treated with a bath of ethyl acetate (a solvent) and the precipitating bath be water since ethyl acetate is only partially miscible in said bath. Material carrying ethyl cellulose in precipitated form may be treated with a bath of (by volume) acetone 80% and naphtha 20% and the precipitating bath be water since the naphtha is nearly immiscible therein.

45 50 55 Other examples of mixtures of liquids that might be used for the solvent bath are alcohol or acetone or methyl ethyl ketone etc. together with one or more of the following, ethyl acetate, castor oil, butyl alcohol, toluol, gasoline, butyl acetate, carbontetrachloride to be used in connection with a precipitating bath of water.

60 65 70 The solvent bath, the precipitating bath, the times of immersion therein, and such factors will, of course, be varied to meet the particular conditions as will be understood by those skilled in the

75 art. The time in the solvent bath must be so regulated that the solvent action is not prolonged sufficiently to not only dissolve but also to remove from the fabric the colloidal matter. The above examples are given merely as illustrations, as the percentages of the restraining agent in the bath may be varied to meet the particular conditions.

80 85 90 Generally speaking, for a Lovell material having e. g. flannel for a base and carrying about 6 ounces of precipitated cellulose nitrate per square yard, I find that twelve seconds treatment with a mixture containing 80% ethyl alcohol and 20% toluol as mentioned above, followed by immersion for 15 minutes in water will give the desired result. In any case, in consideration of the result desired, and as here illustrated, the time of immersion in the precipitating bath is so correlated with the amount and efficacy of the particular restraining agent used that the restraining agent will, for the full length of the period of immersion in the precipitating bath, prevent the precipitation of more than a part only of the colloidal matter. As will be understood by those skilled in the art, these factors may be widely varied to meet the circumstances of different particular cases.

95 100 While boots and shoes have been more particularly referred to, it will be understood that stiffeners of the present type may be used in any article of footwear, where the use recommends itself, and furthermore, may be used in any particular location desired as in the toe to form the box or in the heel to form the counter.

105 110 As will be evident the production of the stiffening material in accordance with Lovell and its treatment in accordance with the present invention, may be carried on as a single continuous process.

I claim:

1. Method comprising treating a fabric whose interstices carry a precipitated cellulose derivative, with a solvent-liquid to dissolve the cellulose derivative without removing it from the fabric, passing the fabric without drying into a precipitating bath, said solvent-liquid and said precipitating bath being at least partially immiscible and the fabric being subjected to said precipitating bath for a period of time only sufficient to precipitate part of the cellulose derivative, drying the fabric, and thereafter treating said fabric with a cellulose derivative solvent to soften it, shaping it, and allowing it to dry in the desired final form. 40 45 50

2. Method comprising treating a fabric whose interstices carry a precipitated cellulose derivative, with a solvent-liquid to dissolve the cellulose derivative without removing it from the fabric, said solvent-liquid comprising a water-soluble solvent for the cellulose derivative and a water-immiscible liquid, passing the fabric without drying into a water bath, the fabric being subjected to said water bath for a period of time only sufficient to precipitate part of the cellulose derivative, drying the fabric, and thereafter treating said fabric with a cellulose derivative solvent to 55 60 65 soften it, shaping it, and allowing it to dry in the desired final form.

3. Method comprising treating a fabric whose interstices carry precipitated cellulose nitrate, with a solvent-liquid to dissolve the cellulose nitrate without removing it from the fabric, passing the fabric without drying into a precipitating bath, said solvent-liquid and said precipitating bath being at least partially immiscible, the fabric being subjected to said precipitating bath 70 75 80

- for a period of time only sufficient to precipitate part of the cellulose nitrate, drying the fabric, and thereafter treating said fabric with a cellulose nitrate solvent to soften it, shaping it, and allowing it to dry in the desired final form.

4. Method comprising treating a fabric whose interstices carry precipitated cellulose nitrate, with a solvent-liquid to dissolve the cellulose nitrate without removing it from the fabric, said solvent-liquid comprising a water-soluble solvent for the cellulose nitrate and a water-immiscible liquid, passing the fabric without drying into a water bath, the fabric being subjected to said water bath for a period of time only sufficient to precipitate part of the cellulose nitrate, drying the fabric, and thereafter treating said fabric with a cellulose nitrate solvent to soften it, shaping it, and allowing it to dry in the desired final form.

10 5. Method comprising treating a fabric whose interstices carry precipitated cellulose nitrate, with a solvent-liquid to dissolve the cellulose nitrate without removing it from the fabric, said solvent-liquid comprising a water-soluble solvent for the cellulose nitrate and a water-immiscible liquid from the group consisting of castor oil and toluol, passing the fabric without drying into a water bath, the fabric being subjected to said water bath for a period of time only sufficient to precipitate part of the cellulose nitrate, drying the fabric, and thereafter treating said fabric with a cellulose nitrate solvent to soften it, shaping it, and allowing it to dry in the desired final form.

15 6. Method comprising treating a fabric whose interstices carry precipitated cellulose acetate, with a solvent-liquid to dissolve the cellulose acetate without removing it from the fabric, said solvent-liquid comprising a water-soluble solvent for the cellulose acetate and a water-immiscible liquid, passing the fabric without drying into a water bath, the fabric being subjected to said water bath for a period of time only sufficient to precipitate part of the cellulose acetate, drying the fabric, and thereafter treating said fabric with a cellulose acetate solvent to soften it, shaping it, and allowing it to dry in the desired final form.

20 7. Method comprising treating a fabric whose interstices carry precipitated cellulose ether, with a solvent-liquid to dissolve the cellulose ether without removing it from the fabric, said solvent-liquid comprising a water-soluble solvent for the cellulose ether and a water-immiscible liquid, passing the fabric without drying into a water bath, the fabric being subjected to said water bath for a period of time only sufficient to precipitate part of the cellulose ether, drying the fabric, and thereafter treating said fabric with a cellulose ether solvent to soften it, shaping it, and allowing it to dry in the desired final form.

25 8. Method comprising treating a fabric whose interstices carry precipitated ethyl cellulose, with a solvent liquid to dissolve the ethyl cellulose without removing it from the fabric, said solvent liquid comprising a water-soluble solvent for the ethyl cellulose and a water-immiscible liquid, passing the fabric without drying into a water bath, the fabric being subjected to said water bath for a period of time only sufficient to precipitate part of the ethyl cellulose, drying the fabric, and thereafter treating said fabric with an ethyl cellulose solvent to soften it, shaping it, and allowing it to dry in the desired final form.

30 9. A stiffening blank comprising a fabric whose interstices carry cellulosic derivative in precipitated form, the fabric also carrying, distributed uniformly throughout the precipitated derivative, cellulosic derivative in a relatively firmer, harder, colloided, and more solvent-resistant form, said blank being adapted to be treated with a cellulose derivative solvent to soften same, and then shaped and dried in the desired final form.

35 10. A stiffening blank comprising a fabric whose interstices carry cellulose acetate in precipitated form, the fabric also carrying, distributed uniformly throughout the precipitated cellulose acetate, cellulose acetate in a relatively firmer, harder, colloided, and more solvent-resistant form, said blank being adapted to be treated with a cellulose acetate solvent to soften same, and then shaped and dried in the desired final form.

40 11. A stiffening blank comprising a fabric whose interstices carry cellulose nitrate in precipitated form, the fabric also carrying, distributed uniformly throughout the precipitated cellulose nitrate, cellulose nitrate in a relatively firmer, harder, colloided, and more solvent-resistant form, said blank being adapted to be treated with a cellulose nitrate solvent to soften same, and then shaped and dried in the desired final form.

45 12. A stiffening blank comprising a fabric whose interstices carry cellulose ether in precipitated form, the fabric also carrying, distributed uniformly throughout the precipitated cellulose ether, cellulose ether in a relatively firmer, harder, colloided, and more solvent-resistant form, said blank being adapted to be treated with a cellulose ether solvent to soften same, and then shaped and dried in the desired final form.

50 13. A stiffening blank comprising a fabric whose interstices carry ethyl cellulose in precipitated form, the fabric also carrying, distributed uniformly throughout the precipitated ethyl cellulose, ethyl cellulose in a relatively firmer, harder, colloided, and more solvent-resistant form, said blank being adapted to be treated with an ethyl cellulose solvent to soften same, and then shaped and dried in the desired final form.

55 14. Method comprising treating a fabric whose

## EARLE H. CAMERON.